



US009983491B2

(12) **United States Patent**  
**Onishi et al.**

(10) **Patent No.:** **US 9,983,491 B2**  
(b4) **Date of Patent:** **May 29, 2018**

(54) **PROCESS FOR PRODUCING A TONER**(71) Applicant: **Konica Minolta, Inc.**, Tokyo (JP)(72) Inventors: **Junya Onishi**, Tokyo (JP); **Shiro Hirano**, Tokyo (JP); **Noboru Ueda**, Tokyo (JP); **Kouji Sugama**, Tokyo (JP); **Aya Shirai**, Tokyo (JP)(73) Assignee: **KONICA MINOLTA, INC.**, Tokyo (JP)

(\* ) Notice: Subject to any disclaimer, the term of this patent is extended or adjusted under 35 U.S.C. 154(b) by 0 days. days.

(21) Appl. No.: **15/439,435**(22) Filed: **Feb. 22, 2017**(65) **Prior Publication Data**

US 2017/0255114 A1 Sep. 7, 2017

(30) **Foreign Application Priority Data**

Mar. 1, 2016 (JP) ..... 2016-038844

(51) **Int. Cl.**  
**G03G 9/08** (2006.01)(52) **U.S. Cl.**  
CPC ..... **G03G 9/0804** (2013.01); **G03G 9/0815** (2013.01); **G03G 9/0825** (2013.01)(58) **Field of Classification Search**  
CPC ... G03G 9/0804; G03G 9/081; G03G 9/0815;  
G03G 9/0825

See application file for complete search history.

(56) **References Cited**

## U.S. PATENT DOCUMENTS

7,494,757 B2 2/2009 Sacripante et al.  
2003/0049554 A1\* 3/2003 Ohmura ..... G03G 9/0804  
430/110.2

2003/0104296 A1\* 6/2003 Hamano ..... G03G 9/0804  
430/107.1  
2007/0254229 A1\* 11/2007 Patel ..... G03G 9/0804  
430/108.4  
2011/0086302 A1\* 4/2011 Zhou ..... G03G 9/0804  
430/105  
2013/0209931 A1\* 8/2013 Sato ..... G03G 9/0804  
430/109.4  
2014/0302437 A1\* 10/2014 Shimano ..... G03G 9/0806  
430/137.15  
2014/0356780 A1\* 12/2014 Kawamura ..... G03G 9/08724  
430/109.3

## FOREIGN PATENT DOCUMENTS

|    |              |         |
|----|--------------|---------|
| JP | 2001222138 A | 8/2001  |
| JP | 2009063992 A | 3/2009  |
| JP | 2012042508 A | 3/2012  |
| JP | 2012098697 A | 5/2012  |
| JP | 2014211632 A | 11/2014 |

\* cited by examiner

Primary Examiner — Christopher D RoDee

(74) Attorney, Agent, or Firm — Lucas &amp; Mercanti, LLP

(57) **ABSTRACT**

A process for producing a toner of the present invention includes: a first step of heating a dispersion containing an aqueous medium and a binder resin containing a crystalline resin to a temperature higher than or equal to a melting point of the crystalline resin; and a second step of maintaining the dispersion at temperature T (° C.) for 30 minutes or longer in a state where a pH of the dispersion is maintained at 5.5 or higher and 9.0 or lower, in which the temperature T satisfies the following expression,  $R_c - 25 \leq T \leq R_c - 5$ , where the  $R_c$  represents a recrystallization temperature (° C.) of the crystalline resin.

**16 Claims, 1 Drawing Sheet**



FIG. 1A



FIG. 1D



FIG. 1B



FIG. 1E



FIG. 1C



FIG. 1F

## PROCESS FOR PRODUCING A TONER

## CROSS REFERENCE TO RELATED APPLICATIONS

This application is entitled to and claims the benefit of Japanese Patent Application No. 2016-038844, filed on Mar. 1, 2016, the disclosure of which including the specification, drawings and abstract is incorporated herein by reference in its entirety.

## BACKGROUND OF THE INVENTION

## 1. Field of the Invention

The present invention relates to a process for producing a toner for development of electrostatic images.

## 2. Description of Related Art

To increase printing speed and achieve further saving of energy for reduction of environmental loads in electrophotographic image forming apparatuses, a toner for development of electrostatic images (hereinafter, simply referred to as "toner") which is capable of heat fixing at lower temperatures has been recently required. Such a toner needs lowering of the melting temperature and melt viscosity of a binder resin, and a toner having low-temperature fixability enhanced by adding a crystalline resin such as a crystalline polyester resin is suggested (e.g., see Japanese Patent Application Laid-Open No. 2001-222138). When a toner containing a crystalline resin is heated to a temperature higher than or equal to the melting point of the crystalline resin in production of the toner, however, the crystalline resin becomes compatible with an amorphous resin even in production, which inconveniently deteriorates the high-temperature storability.

Annealing (hereinafter, also referred to as heat treatment) is known as means for enhancing the high-temperature storability of a toner having such a composition. For example, it is reported that heat treatment at a temperature higher than or equal to the glass transition temperature of an amorphous resin and lower than or equal to the melting point of a crystalline resin—10° C. for a long duration allows the crystalline resin which is compatible with the amorphous resin to recrystallize to enhance the high-temperature storability (e.g., see Japanese Patent Application Laid-Open No. 2009-063992).

In addition, there is known a method of controlling the heating/retaining temperature for an aqueous dispersion of a crystalline resin of a block polymer (e.g., see Japanese Patent Application Laid-Open No. 2014-211632). According to the document, this method enables control of the crystalline resin domain even in recrystallization of the crystalline resin, and thus the crystalline resin domain can be finely dispersed to prevent deterioration of fixability.

Further, it is reported that heating and retaining of a toner composition containing a binder resin containing a crystalline polyester under predetermined conditions allows the toner to keep the low-temperature fixability and high-temperature storability for a long period (e.g., see Japanese Patent Application Laid-Open No. 2012-42508). Furthermore, a method is known in which a differential scanning colorimetry curve is obtained in measurement for a crystalline polyester resin by using a differential scanning colorimeter and heat treatment is performed at the onset temperature  $\pm 5^\circ \text{C}$ . of an endothermic peak in the curve (e.g., see Japanese Patent Application Laid-Open No. 2012-98697). Moreover, there is known heat treatment of a toner particle containing a crystalline resin and an amorphous resin at a

temperature which is higher than or equal to the glass transition temperature of the crystalline resin and is the recrystallization temperature  $\pm 10^\circ \text{C}$ . (e.g., see U.S. Pat. No. 7,494,757).

In dry heat treatment, however, the elevation of the glass transition temperature, the increase of the domain diameter of a crystalline resin in a toner, etc., are caused due to the change of the moisture adsorption state of a toner, and this makes it difficult to exhibit low-temperature fixing performance at a level required in recent years. Also, when heat treatment is conducted in an aqueous medium, a crystalline resin may be exposed in a surface of a toner. The exposure of a crystalline resin in a surface of a toner may lower surface resistance of the toner and/or deteriorate charging characteristics of the toner, resulting in an image noise, such as density unevenness of images.

Thus, in a related-art process for production of a toner, there remains room for a further investigation from the viewpoint of achieving low-temperature fixability of a toner and suppressing density unevenness of images to be obtained.

## SUMMARY OF THE INVENTION

An object of the present invention is to provide a toner which has excellent low-temperature fixability and is capable of suppressing density unevenness of images to be obtained.

The present inventors have found that proper control of a domain diameter and a presence state of a crystalline resin in a toner is important to obtain a toner which has excellent low-temperature fixability and is capable of suppressing density unevenness of images. Further, in a process for production of a toner by an emulsion aggregation method in which a toner base particle is produced by aggregating and fusing fine particles of a binder resin containing a crystalline resin in the presence of a metal ion, a presence state and a domain diameter of the crystalline resin in a toner have been found to be accurately controllable by controlling both a heat treatment scheme of a dispersion containing the toner base particle and a pH of the dispersion during heat treatment. The present invention was made on the basis of such findings.

In order to achieve the object mentioned above, a process for producing a toner, reflecting one aspect of the present invention includes: a first step of heating a dispersion containing an aqueous medium and a binder resin containing a crystalline resin to a temperature higher than or equal to a melting point of the crystalline resin in a production step for forming a toner base particle by aggregating and fusing a fine particle of the binder resin containing the crystalline resin in the presence of a metal ion; and a second step of maintaining the dispersion at temperature T (° C.) for 30 minutes or longer in a state where a pH of the dispersion is maintained at 5.5 or higher and 9.0 or lower, in which the temperature T satisfies the following expression,  $Rc-25 \leq T \leq Rc-5$ , where the Rc represents a recrystallization temperature (° C.) of the crystalline resin.

## BRIEF DESCRIPTION OF DRAWINGS

The present invention will become more fully understood from the detailed description given hereinbelow and the appended drawings which are given by way of illustration only, and thus are not intended as a definition of the limits of the present invention, and wherein:

FIG. 1A is a graph showing a first example of the temperature change of a dispersion from after the end of the first step to the end of the second step of the present invention;

FIG. 1B is a graph showing a second example of the temperature change of a dispersion from after the end of the first step to the end of the second step of the present invention;

FIG. 1C is a graph showing a third example of the temperature change of a dispersion from after the end of the first step to the end of the second step of the present invention;

FIG. 1D is a graph showing a fourth example of the temperature change of a dispersion from after the end of the first step to the end of the second step of the present invention;

FIG. 1E is a graph showing a fifth example of the temperature change of a dispersion from after the end of the first step to the end of the second step of the present invention; and

FIG. 1F is a graph showing a sixth example of the temperature change of a dispersion from after the end of the first step to the end of the second step of the present invention;

#### DESCRIPTION OF THE PREFERRED EMBODIMENTS

In the following, embodiments of the present invention will be described.

A process for producing a toner according to the present embodiment includes: 1) a first step of heating a dispersion containing an aqueous medium and a binder resin containing a crystalline resin to a temperature higher than or equal to a melting point of the crystalline resin in a production step for forming a toner base particle by aggregating and fusing a fine particle of the binder resin containing the crystalline resin in the presence of a metal ion; and 2) a second step of maintaining the dispersion at temperature T (° C.) for 30 minutes or longer in a state where a pH of the dispersion is maintained at 5.5 or higher and 9.0 or lower, in which the temperature T satisfies the following expression,  $Rc-25 \leq T \leq Rc-5$ , where the Rc represents a recrystallization temperature (° C.) of the crystalline resin.

Each step will be described in the following.

##### [First Step]

The first step is a step of heating a dispersion containing the binder resin and an aqueous medium to a temperature higher than or equal to a melting point (Tm) of the crystalline resin in the toner base particle. The temperature of the dispersion in the first step is not limited and may be any temperature higher than or equal to a melting point of the crystalline resin, and the upper limit is the boiling point of the aqueous medium (e.g., the boiling point of water). For heating the dispersion, a known heating apparatus such as a heater may be used. The melting point of the crystalline resin can be measured in differential scanning calorimetry (hereinafter, also simply referred to as DSC) to be described later.

##### [Aqueous Medium]

The aqueous medium refers to a medium having a water content of 50 mass % or more. Examples of components other than water include water-soluble organic solvents such as methanol, ethanol, isopropanol, butanol, acetone, methyl ethyl ketone, and tetrahydrofuran. Among them, alcohol organic solvents which do not dissolve resins therein are particularly preferred, such as methanol, ethanol, isopropanol, and butanol.

##### [Toner Base Particle]

The toner base particle is formed by aggregating and fusing fine particles of a binder resin containing a crystalline resin in the presence of a metal ion. For example, dispersing fine particles of a binder resin containing a crystalline resin and an aggregating agent to be described below in an aqueous medium, and heating the prepared dispersion can aggregate and fuse the fine particles of the binder resin.

##### [Aggregating Agent]

In a process for producing a toner according to the present embodiment, an aggregating agent is used for aggregating fine particles of the binder resin. The aggregating agent may be selected from metal salts in the light of growing particles by charge neutralization reaction and crosslinking action.

Examples of the metal salts include salts of monovalent metals including alkali metals, such as sodium, potassium, and lithium; salts of divalent metals, such as calcium, magnesium, manganese, and copper; and salts of trivalent metals such as iron and aluminum. Specific examples of the metal salts include sodium chloride, potassium chloride, lithium chloride, calcium chloride, magnesium chloride, zinc chloride, copper sulfate, magnesium sulfate, and manganese sulfate. Among them, it is particularly preferred to use salts of divalent metals because they can promote aggregation in a smaller amount. One of them may be used singly, or two or more thereof may be used in combination.

The aggregating agent added allows fine particles of a binder resin to bond together through ionic crosslinking in the aqueous medium, and thus the presence state of the crystalline resin can be more advantageously controlled in heat treatment.

The growth of an aggregated particle can be substantially terminated by raising the salt concentration of an aqueous medium. For example, sodium chloride, or a polyvalent organic acid or a salt thereof, an amino acid or a salt thereof, a polyphosphonic acid or a salt thereof may be used as an aggregation terminator. Alternatively, aggregating action can be reduced by changing the pH in the system. For pH adjustment, for example, an aqueous solution of sodium fumarate, an aqueous solution of sodium hydroxide, or hydrochloric acid, may be used. In addition, use of a chelating agent in combination with pH adjustment is also effective for reducing crosslinking action of a metal ion. Examples of such chelating agents include HIDA (hydroxyethyliminodiacetic acid), HEDTA (hydroxyethylethylenediaminetriacetic acid), HEDP (hydroxyethylidenediphosphonic acid), and HIDS (3-hydroxy-2,2'-iminodisuccinic acid).

The average circularity of a toner base particle to be obtained can be controlled in an aging step for aging of a toner base particle. In an aging step, a dispersion of a toner base particle is heated to age the toner base particle until an intended average circularity of the toner base particle is obtained.

The toner base particle may have a core-shell structure. In the case that a toner base particle having a core-shell structure is formed, a shell layer is formed on the surface of a toner base particle as a core particle. Specifically, a resin to constitute a shell layer is dispersed in an aqueous medium to prepare a resin particle dispersion, which is added to a dispersion of a toner base particle obtained in a formation step or aging step for a toner base particle to aggregate and fuse the resin particle as a shell layer on the surface of the toner base particle. In this way, a dispersion of a toner base particle having a core-shell structure can be obtained. To aggregate and fuse the resin particles as the shell layer on the core particle more strongly, heat treatment may be performed after the shell formation step. Heat treatment is

## 5

suitably performed until an intended average circularity of the toner base particle is obtained.

For aggregation/fusion reaction, an additional toner material other than the binder resin may be further added to the dispersion of the fine particles of the binder resin, as long as the advantageous effects of the present embodiment are exerted. Examples of toner materials other than the binder resin include a coloring agent, a release agent, a charging-controlling agent, and a surfactant, each to be described later. One or more of the additional components may be contained. In the case that an additional toner material is added, a dispersion separately prepared and containing a fine particle of an additional toner material such as a coloring agent may be mixed with the dispersion containing the fine particles of the binder resin for the aggregation/fusion reaction.

Although the toner base particle produced as described above may be taken out of the dispersion before being subjected to a later step, the toner base particle is preferably subjected to a later step while being kept in the dispersion.

## [Fine Particle of Binder Resin]

The fine particles of the binder resin can be produced by using an emulsion polymerization method in which a monomer of a resin is added to an aqueous medium together with a polymerization initiator and the monomer is allowed to undergo polymerization reaction to obtain a dispersion of resin particles. The emulsion polymerization method can be performed in multiple stages. In the case of polymerization reaction in three stages, for example, a dispersion of resin particles is prepared in the first stage of polymerization, and a monomer of a resin and a polymerization initiator are further added in the dispersion for the second stage of polymerization. To the dispersion prepared in the second stage of polymerization, a monomer of a resin and a polymerization initiator are further added for the third stage of polymerization. In the second and third stages of polymerization, a newly added monomer can be additionally polymerized with the resin particles generated in the previous polymerization, as seeds, in the dispersion, and thus the particle size, etc., of the resin particles can be made uniform. Use of a different monomer in each stage of polymerization reaction can provide the resin particles with a multilayer structure and readily provide resin particles having intended characteristics.

## (Polymerization Initiator)

A known polymerization initiator may be used in the polymerization reaction, and examples thereof include persulfates such as ammonium persulfate, sodium persulfate, and potassium persulfate; azo compounds such as 2,2'-azobis(2-aminodipropane) hydrochloride, 2,2'-azobis-(2-aminodipropane) nitrate, 4,4'-azobis-4-cyanovaleic acid, and poly(tetraethylene glycol-2,2'-azobisisobutyrate); and peroxides such as hydrogen peroxide. The amount of the polymerization initiator to be added depends on intended molecular weight and molecular weight distribution, and specifically, can be 0.1 to 5.0 mass % based on the amount of a polymerizable monomer added.

## (Chain Transfer Agent)

A chain transfer agent may be added in the polymerization reaction from the viewpoint of controlling the molecular weight of the resin particles. Examples of chain transfer agents which can be used include mercaptans such as octyl mercaptan; and mercaptopropionates such as n-octyl 3-mercaptopropionate. The amount of the chain transfer agent to be added depends on intended molecular weight and

## 6

molecular weight distribution, and specifically, can be 0.1 to 5.0 mass % based on the amount of a polymerizable monomer added.

## (Surfactant)

5 A surfactant may be added in the polymerization reaction from the viewpoint of preventing the aggregation of the resin fine particle in the dispersion, etc., to maintain a satisfactory dispersion state. Examples of such surfactants include known surfactants including cationic surfactants such as dodecylammonium bromide and dodecytrimethylammonium bromide; anionic surfactants such as sodium stearate, sodium lauryl sulfate (sodium dodecyl sulfate), and sodium dodecylbenzenesulfonate; and nonionic surfactants such as dodecyl polyoxyethylene ether and hexadecyl polyoxyethylene ether. One of them may be used singly, or two or more thereof may be used in combination.

## [Second Step]

20 The second step is a step of maintaining the dispersion obtained in the first step at temperature T (° C.) for 30 minutes or longer in a state where a pH of the dispersion is maintained at 5.5 or higher and 9.0 or lower, in which the temperature T satisfies the following expression,  $Rc-25 \leq T \leq Rc-5$ , where the Rc represents a recrystallization temperature (° C.) of the crystalline resin (hereinafter, simply referred to as "heat treatment").

25 This means, in the second step, the temperature of the dispersion is maintained at a temperature higher than or equal to  $Rc-25$  ° C. and lower than or equal to  $Rc-5$  ° C. for 30 minutes or longer in a state where a pH of the dispersion is maintained at 5.5 or higher and 9.0 or lower.

30  $Rc$ , which is a temperature at which crystallization of a crystalline resin progresses at the greatest level, is a value determined as a peak top temperature of an exothermic peak in a measurement curve obtained in a temperature-lowering operation in DSC in which the temperature of a crystalline resin is raised from room temperature to 100° C. at a temperature-elevating rate of 10° C./min, retained for 1 minute, and lowered to 0° C. at a temperature-lowering rate of 0.1° C./min. The reason for setting the temperature-lowering rate to 0.1° C./min is that the crystallization temperature obtained at a temperature-lowering rate as low as possible is highly correlated with the performance of a toner obtained by using the process for producing a toner according to the present embodiment and the temperature-lowering rate of 0.1° C./min provides a sufficient correlation.

35 During the heat treatment, as long as temperature T (° C.) of the dispersion satisfies  $Rc-25 \leq T \leq Rc-5$ , a mode of the temperature change of the dispersion from the start to the end of the heat treatment is not limited. For example, the temperature of the dispersion during the heat treatment may be maintained constant, kept elevating or lowering at a constant rate, or constantly changed by repeated elevation and lowering or the like.

40 When a pH of the dispersion during the heat treatment is lower than 5.5, bleeding out of a crystalline resin into the vicinity of a surface of a toner base particle occurs due to a low amount of ionic crosslinking among aggregated fine particles of a binder resin, and charging characteristics and so forth of a toner deteriorate, resulting in density unevenness of images to be obtained. In contrast, when a pH of the dispersion during the heat treatment is higher than 9.0, an amount of ionic crosslinking among aggregated fine particles of a binder resin increases excessively and deteriorates 45 low-temperature fixability of a toner.

From the viewpoint of enhancing low-temperature fixability of a toner and suppressing density unevenness of images, a pH of the dispersion during the heat treatment is preferably 6.0-8.0.

When a pH of the dispersion is 5.5 or higher and 9.0 or lower at the time of completion of the first step, no pH adjustment of the dispersion is needed. When a pH of the dispersion is lower than 5.5, the pH may be adjusted to 5.5 or higher and 9.0 or lower by a known method, such as addition of a sodium hydroxide solution. When a pH of the dispersion is higher than 9.0, the pH may be adjusted to 5.5 or higher and 9.0 or lower by a known method, such as addition of a hydrochloric acid solution.

The pH of the dispersion is measured using, for example, a glass electrode-type pH meter (from DKK-TOA Corporation) at a pre-heat treatment step temperature.

In addition, temperature  $T$  of the heat treatment preferably satisfies  $Rc-25 \leq T \leq Rc-10$  from the viewpoint of the enhancement of the low-temperature fixability and suppressed density unevenness of images. Moreover, the duration of the heat treatment may be 30 minutes or longer, and the upper limit of the duration of the heat treatment may preferably be about 180 minutes from the viewpoint of production efficiency although the upper limit is not particularly limited. Further, heat treatment in an aqueous medium can suppress change in adsorption state of water molecules in a toner and consequently suppress elevation of a glass transition temperature of a binder resin.

[Cooling Step]

A dispersion, obtained in the first step, having been heated to a temperature higher than  $Rc$  may be adjusted to a temperature lower than  $Rc$  (pre-heat treatment step temperature) at an arbitrary temperature-lowering rate by, for example, spontaneous cooling. From the viewpoint of suppressing density unevenness of images, the dispersion is more preferably cooled to a temperature lower than  $Rc-25^\circ C$ .

In the cooling step, it is preferable to rapidly cool the dispersion having been heated to a temperature higher than  $Rc$  at a temperature-lowering rate (cooling rate) of  $1^\circ C./min$  or higher to a temperature lower than  $Rc$ . During this, the dispersion may be cooled at a temperature-lowering rate of  $1^\circ C./min$  or higher at  $Rc$ . Before conducting the second step, cooling the dispersion having been heated to a temperature higher than  $Rc$  so that a temperature-lowering rate at  $Rc$  is  $1^\circ C./min$  or higher can better control a domain diameter and a presence state of a crystalline resin in a toner. Accordingly, low-temperature fixability of a toner to be obtained can be further enhanced and density unevenness of images can be suppressed as well.

“The temperature of the dispersion having been heated to a temperature higher than  $Rc$ ” may be the temperature at the end of the first step, or a predetermined temperature higher than  $Rc$  to which the dispersion is cooled from the temperature at the end of the first step. Accordingly, the dispersion having been heated in the first step may be immediately cooled to a temperature lower than  $Rc$  at a temperature-lowering rate of  $1^\circ C./min$  or higher, or the dispersion may be cooled to a predetermined temperature higher than  $Rc$  at an arbitrary cooling rate and then cooled to a temperature lower than  $Rc$  at a temperature-lowering rate of  $1^\circ C./min$  or higher. In addition, the cooling rate after reaching  $Rc$  is not limited. For example, the cooling rate may be controlled to lower than  $1^\circ C./min$  after the dispersion is cooled to a predetermined temperature lower than  $Rc$  at a temperature-lowering rate of  $1^\circ C./min$  or higher.

The dispersion can be cooled by using a known cooler capable of providing the above cooling rate. For example, an outer bath of a reaction vessel may be quickly cooled, or the dispersion may be allowed to pass through a heat exchanger, or cooled deionized water may be fed into the dispersion. From the viewpoint of production efficiency, cooling with a heat exchanger is preferred.

The cooling rate at  $Rc$  for the dispersion is preferably  $2^\circ C./min$  or higher from the viewpoint of the further enhancement of the low-temperature fixability of the toner. From the viewpoint of the further enhancement of the low-temperature fixability of the toner, the higher the cooling rate is, the better it is, so the cooling rate is more preferably  $5^\circ C./min$  or higher. If the cooling rate is too high, however, few crystal nuclei are formed in cooling and crystallization progresses more slowly, and thus the upper limit of the cooling rate is preferably  $25^\circ C./min$  or lower from the viewpoint of productivity.

[Description of Temperature Change of Dispersion from after End of First Step to End of Second Step]

Examples of the temperature change of the dispersion from after the end of the first step to the end of the second step of the present embodiment will be described in the following with reference to FIGS. 1A to 1F. In the accompanying drawings,  $T$  indicates a temperature region of higher than or equal to  $Rc-25^\circ C$ . and lower than or equal to  $Rc-5^\circ C$ .,  $t$  indicates a duration of 30 minutes or longer,  $A$  indicates a zone of the step of cooling where cooling rate is  $1^\circ C./min$  or higher, and a shaded area indicates a duration and a temperature range of the second step. In the shaded area, as mentioned above, a pH of the dispersion is 5.5 or higher and 9.0 or lower.

In the first example, as illustrated in FIG. 1A, (1) the dispersion having been heated to a temperature higher than  $Rc$  in the first step is cooled to a predetermined temperature lower than  $Rc$  (pre-heat treatment temperature) at a cooling rate of  $1^\circ C./min$  or higher, (2) the dispersion is then cooled to a heat treatment initiation temperature in the temperature region  $T$  at a cooling rate of lower than  $1^\circ C./min$ , and (3) finally the temperature of the dispersion is retained at the heat treatment initiation temperature for the duration  $t$  (the second step).

In the second example, as illustrated in FIG. 1B, (1) the dispersion having been heated to a temperature higher than  $Rc$  in the first step is cooled to a predetermined temperature lower than  $Rc$  (pre-heat treatment temperature) at a cooling rate of  $1^\circ C./min$  or higher, (2) the dispersion is then cooled continuously at a cooling rate of lower than  $1^\circ C./min$  and maintained within the temperature region  $T$  for the duration  $t$  (the second step). In the second example, in contrast to the first example, the temperature of the dispersion is lowered at a constant rate in the second step.

In the third example, as illustrated in FIG. 1C, (1) the dispersion having been heated to a temperature higher than  $Rc$  in the first step is cooled to a predetermined temperature lower than  $Rc$  (pre-heat treatment temperature) at a cooling rate of  $1^\circ C./min$  or higher, (2) the dispersion is then cooled to a heat treatment initiation temperature in the temperature region  $T$  at a cooling rate of lower than  $1^\circ C./min$ , and (3) finally the dispersion is repeatedly heated and cooled to elevate and lower the temperature of the dispersion repeatedly in a manner such that the temperature of the dispersion is maintained within the temperature region  $T$  for the duration  $t$  (the second step). In contrast to the first example and the second example, the temperature of the dispersion is repeatedly elevated and lowered in the second step.

In the fourth example, as illustrated in FIG. 1D, (1) the dispersion having been heated to a temperature higher than  $R_c$  in the first step is cooled to a temperature lower than  $R_c-25^\circ C.$  (pre-heat treatment temperature) at a cooling rate of  $1^\circ C./min$  or higher, (2) the dispersion is then heated to a heat treatment initiation temperature within the temperature region  $T$ , and (3) finally the temperature of the dispersion is retained at the heat treatment initiation temperature for the duration  $t$  (the second step). In contrast to the first example, the dispersion having a temperature higher than  $R_c$  is cooled to a temperature lower than  $R_c-25^\circ C.$  at a cooling rate of  $1^\circ C./min$  or higher, and then heated to the heat treatment initiation temperature.

In the fifth example, as illustrated in FIG. 1E, (1) the dispersion having been heated to a temperature higher than  $R_c$  in the first step is cooled to a temperature lower than  $R_c-25^\circ C.$  (pre-heat treatment temperature) at a cooling rate of  $1^\circ C./min$  or higher, (2) the dispersion is then heated to a heat treatment initiation temperature of  $R_c-5^\circ C.$ , and (3) finally the dispersion is continuously cooled in a manner such that the temperature of the dispersion is maintained within the temperature region  $T$  for the duration  $t$  (the second step). In contrast to the second example, the dispersion having a temperature higher than  $R_c$  is cooled to a temperature lower than  $R_c-25^\circ C.$  at a cooling rate of  $1^\circ C./min$  or higher, and then heated to the heat treatment initiation temperature.

In the sixth example, as illustrated in FIG. 1F, (1) the dispersion having been heated to a temperature higher than  $R_c$  in the first step is cooled to a temperature lower than  $R_c-25^\circ C.$  (pre-heat treatment temperature) at a cooling rate of  $1^\circ C./min$  or higher, (2) the dispersion is then heated to a heat treatment initiation temperature within the temperature region  $T$ , and (3) finally the dispersion is repeatedly heated and cooled to elevate and lower the temperature of the dispersion repeatedly in a manner such that the temperature of the dispersion is maintained within the temperature region  $T$  for the duration  $t$  (the second step). In contrast to the third example, the dispersion having a temperature higher than  $R_c$  is cooled to a temperature lower than  $R_c-25^\circ C.$  at a cooling rate of  $1^\circ C./min$  or higher, and then heated to the heat treatment initiation temperature.

Thus, in the process for producing a toner according to the present embodiment, in a production step of a toner base particle by an emulsion aggregation method in the presence of a metal ion, the temperature of the dispersion containing an aqueous medium and a binder resin containing a crystalline resin is maintained within the range of  $R_c-25^\circ C.$  or higher and  $R_c-5^\circ C.$  or lower for 30 minutes or longer in a state where a pH of the dispersion is maintained at 5.5 or higher and 9.0 or lower.

The process for producing a toner according to the present embodiment may further include an additional step other than the above-described first and second steps, as long as the advantageous effects of the present embodiment are exerted. Examples of the additional step include a step of mixing an external additive with the resultant toner base particle to allow the external additive to attach to the toner base particle to obtain a toner particle, and a step of mixing the resultant toner particle with a carrier particle to obtain a toner as a two-component developer.

#### [Toner]

A toner produced by using the production process according to the present embodiment contains, as described above, a toner base particle at least containing a binder resin, and the toner base particle is a particle primarily composed of a binder resin and, as necessary, containing various additives

such as a coloring agent, a release agent, a charging-controlling agent, and a surfactant. First, the binder resin will be described.

#### [Binder Resin]

The binder resin contains a crystalline resin and an amorphous resin. In the present specification, "the binder resin contains a crystalline resin" may refer to a mode in which the binder resin contains a crystalline resin itself, or may refer to a mode in which the binder resin contains a segment in another resin, as a crystalline polyester polymerization segment in a hybrid crystalline resin to be described later. In the present specification, "the binder resin contains an amorphous resin" may refer to a mode in which the binder resin contains an amorphous resin itself, or may refer to a mode in which the binder resin contains a segment in another resin, as an amorphous resin segment in a hybrid crystalline resin to be described later.

#### (Crystalline Resin)

The crystalline resin is a resin that has a clear endothermic peak, not a stepwise endothermic change, in DSC for a toner. Specifically, a clear endothermic peak refers to an endothermic peak whose full width at half maximum is within  $15^\circ C.$  in DSC carried out at a temperature-elevating rate of  $10^\circ C./min$ . The content of such a crystalline resin is preferably 3 to 30 mass % based on the amount of a toner. This can provide an effect of improving the sharp melting properties of the binder resin to enhance the low-temperature fixability of a toner, and prevent lowering of the heat resistance caused by the crystalline resin contained.

Examples of the crystalline resin include crystalline polyester resins, crystalline polyamide resins, crystalline polyurethane resins, crystalline polyacetal resins, crystalline polyethylene terephthalate resin, crystalline polybutylene terephthalate resin, crystalline polyphenylene sulfide resin, crystalline polyether ether ketone resins, and crystalline polytetrafluoroethylene resin. Among them, crystalline polyester resins are preferred. The reason is that a crystalline polyester resin melts in heat fixation to serve as a plasticizer for an amorphous resin, and thus the low-temperature fixability can be enhanced. Such a crystalline polyester resin can be obtained, for example, by using a known synthesis method through dehydration condensation reaction between a polycarboxylic acid and a polyalcohol. One crystalline polyester resin or more than one crystalline polyester resin may be used.

Examples of the polycarboxylic acid include saturated aliphatic dicarboxylic acids such as succinic acid, sebacic acid, and dodecanedioic acid; alicyclic dicarboxylic acids such as cyclohexanedicarboxylic acid; aromatic dicarboxylic acids such as phthalic acid, isophthalic acid, and terephthalic acid; trivalent or higher polycarboxylic acids such as trimellitic acid and pyromellitic acid; acid anhydrides thereof; and C1-3 alkyl esters thereof. The polycarboxylic acid is preferably an aliphatic dicarboxylic acid.

Examples of the polyalcohol include aliphatic diols such as ethylene glycol, 1,2-propanediol, 1,3-propanediol, 1,4-butanediol, 1,5-pentanediol, 1,6-hexanediol, 1,7-heptanediol, 1,8-octanediol, neopentyl glycol, and 1,4-butenediol; trihydric or higher alcohols such as glycerin, pentaerythritol, trimethylolpropane, and sorbitol. The polyalcohol is preferably an aliphatic diol.

The crystalline polyester resin is preferably a hybrid crystalline resin modified with a styrene-acrylic resin (hereinafter, also simply referred to as "hybrid crystalline resin"). The reason is that the styrene-acrylic resin portion of a hybrid crystalline resin has high compatibility with an amorphous resin and the crystalline polyester resin can be

## 11

uniformly dispersed in the toner base particle; and in the case that the toner base particle has a core-shell structure to be described later and the shell layer contains a hybrid crystalline resin, the styrene-acrylic resin portion tends to aggregate on the surface of the core particle containing an amorphous resin and cover the whole surface of the core particle.

In the present embodiment, "a crystalline polyester resin is modified with a styrene-acrylic resin" refers to a state in which a crystalline polyester resin segment and a styrene-acrylic resin segment chemically bond to each other. A crystalline polyester resin segment refers to a resin portion derived from a crystalline polyester resin, that is, a molecular chain having the same chemical structure as the crystalline polyester resin, in a hybrid crystalline resin. A styrene-acrylic resin segment refers to a resin portion derived from a styrene-acrylic resin, that is, a molecular chain having the same chemical structure as the styrene-acrylic resin, in a hybrid crystalline resin.

The styrene-acrylic resin is a polymer of a styrenic monomer and a (meth)acrylic monomer.

Examples of the styrenic monomer include styrene, o-methylstyrene, m-methylstyrene, p-methylstyrene, p-methoxystyrene, p-phenylstyrene, p-chlorostyrene, p-ethylstyrene, p-n-butylstyrene, p-tert-butylstyrene, p-n-hexylstyrene, p-n-octylstyrene, p-n-nonylstyrene, p-n-decylstyrene, p-n-dodecylstyrene, 2,4-dimethylstyrene, 3,4-dichlorostyrene, and derivatives thereof. One of them may be used singly, or two or more thereof may be used in combination.

Examples of the (meth)acrylic monomer include acrylic acid, methacrylic acid, methyl acrylate, ethyl acrylate, butyl acrylate, 2-ethylhexyl acrylate, cyclohexyl acrylate, phenyl acrylate, methyl methacrylate, ethyl methacrylate, butyl methacrylate, hexyl methacrylate, 2-ethylhexyl methacrylate, ethyl 6-hydroxyacrylate, propyl  $\gamma$ -aminoacrylate, stearyl methacrylate, dimethylaminoethyl methacrylate, diethylaminoethyl methacrylate, 2-hydroxyethyl (meth)acrylate, 2-hydroxypropyl (meth)acrylate, 3-hydroxypropyl (meth)acrylate, 2-hydroxybutyl (meth)acrylate, 3-hydroxybutyl (meth)acrylate, 4-hydroxybutyl (meth)acrylate, and polyethylene glycol mono(meth)acrylate. One of them may be used singly, or two or more thereof may be used in combination.

In addition to the styrenic monomer and the (meth)acrylic monomer, an additional monomer may be used. Examples of the additional monomer which can be used include maleic acid, itaconic acid, cinnamic acid, fumaric acid, monoalkyl maleates, and monoalkyl itaconates.

The styrene-acrylic resin can be obtained by adding an arbitrary common polymerization initiator such as a peroxide, a persulfate, and an azo compound and polymerizing the above-described monomers by a known polymerization method such as bulk polymerization, solution polymerization, an emulsion polymerization method, a miniemulsion method, a suspension polymerization method, and a dispersion polymerization method. In polymerization, a common chain transfer agent such as an alkyl mercaptan and a mercapto fatty acid ester may be used for the purpose of adjusting the molecular weight.

The content of the styrene-acrylic resin segment in the hybrid crystalline resin is preferably 10 mass % or lower from the viewpoint of low-temperature fixability.

The hybrid crystalline resin can be obtained by allowing the crystalline polyester resin and the styrene-acrylic resin each separately prepared to react and chemically bond to each other. From the viewpoint of facilitating bonding, it is

## 12

preferred to incorporate a substituent capable of reacting with both of the crystalline polyester resin and the styrene-acrylic resin into either the crystalline polyester resin or the styrene-acrylic resin. In formation of the styrene-acrylic resin, for example, a compound having a substituent capable of reacting with a carboxy group (COOH) or a hydroxy group (OH) in the crystalline polyester resin and a substituent capable of reacting with the styrene-acrylic resin is added in addition to the styrenic monomer and the (meth)acrylic monomer as raw materials. This provides a styrene-acrylic resin having a substituent capable of reacting with a carboxy group (COOH) or a hydroxy group (OH) in the crystalline polyester resin.

Alternatively, the hybrid crystalline resin can be obtained by performing polymerization reaction in the presence of the crystalline polyester resin prepared in advance to produce the styrene-acrylic resin, or by performing polymerization reaction in the presence of the styrene-acrylic resin prepared in advance to produce the crystalline polyester resin. In both cases, a compound having a substituent capable of reacting with both of the crystalline polyester resin and the styrene-acrylic resin as described above is suitably added in polymerization reaction.

The number average molecular weight ( $M_n$ ) of the hybrid crystalline resin is preferably 2,000 to 10,000 from the viewpoint of fixability.

The melting point of the crystalline resin according to the present embodiment is preferably 50 to 90° C., and more preferably 60 to 80° C. from the viewpoint of obtaining sufficient low-temperature fixability and high-temperature storability.

The melting point of the crystalline resin can be measured in DSC. Specifically, a sample of the crystalline resin is sealed in the aluminum pan KITNO.B0143013, and the pan is attached to a sample holder of the thermal analyzer Diamond DSC (from PerkinElmer Inc.), and the temperature is changed by heating, cooling, and heating, in the order presented. In the first and second heating, the temperature is elevated from room temperature (25° C.) to 150° C. at a temperature-elevating rate of 10° C./min and the temperature is retained at 150° C. for 5 minutes, and in the cooling, the temperature is lowered from 150° C. to 0° C. at a temperature-lowering rate of 10° C./min and the temperature is retained at 0° C. for 5 minutes. A peak top temperature of an exothermic peak in an exothermic curve obtained in the second heating is measured as the melting point.

The content of the crystalline polyester resin in the binder resin is preferably 5 to 50 mass %. If the content of the crystalline polyester resin in the binder resin is less than 5 mass %, the effect on low-temperature fixing may be lowered, and if the content of the crystalline polyester resin in the binder resin is more than 50 mass %, the high-temperature storability may be deteriorated. The content of the crystalline resin in the toner base particle is preferably 1 to 20 mass %, and more preferably 5 to 15 mass % from the viewpoint of obtaining sufficient low-temperature fixability and high-temperature storability. An amorphous vinyl resin to be described later can uniformly disperse the crystalline resin whose content is within this range in a toner particle and sufficiently inhibit crystallization.

It is preferable that the weight average molecular weight ( $M_w$ ) of the crystalline resin according to the present embodiment be 5,000 to 50,000, and the number average molecular weight thereof be 2,000 to 10,000 from the viewpoint of low-temperature fixability and glossiness stability.

The weight average molecular weight and the number average molecular weight can be determined from a molecular weight distribution measured by using gel permeation chromatography (GPC), as in the following.

A sample is added to tetrahydrofuran so that the concentration reaches 1 mg/mL, and dispersed with an ultrasonic disperser at room temperature for 5 minutes, and the resultant dispersion is processed by using a membrane filter with a pore size of 0.2  $\mu$ m to prepare a sample solution. With use of the GPC apparatus HLC-8120GPC (from Tosoh Corporation) and TSKguardcolumn+TSKgel SuperHZ-M of 3 columns coupled in series (from Tosoh Corporation), tetrahydrofuran as a carrier solvent is allowed to flow through at a flow rate of 0.2 mL/min with the column temperature retained at 40° C. Together with the carrier solvent, 10  $\mu$ L of the sample solution prepared is injected into the GPC apparatus. The sample is detected with a refractive index detector (RI detector), and the molecular weight distribution of the sample is calculated by using a calibration curve obtained in measurement for a monodisperse polystyrene standard particle. Ten polystyrenes samples are used for determination of the calibration curve.

(Amorphous Resin)

Amorphous resins are resins with amorphous characteristics of having a glass transition temperature (Tg) but having no melting point or clear endothermic peak when the temperature is elevated, as described above, in an endothermic curve obtained in DSC.

The amorphous resin is used as the binder resin together with the crystalline resin, and constitutes the toner base particle. One amorphous resin or more than one amorphous resin may be used. The amorphous resin may be a vinyl resin, or a urethane resin, a urea resin, an amorphous polyester resin or a partially modified polyester resin, or a combination thereof. The amorphous resin is also available, for example, through a known synthesis method. The amorphous resin is preferably a vinyl resin from the viewpoint of the enhancement of the low-temperature stability and high-temperature storability.

(Amorphous Vinyl Resin)

The amorphous vinyl resin is not limited and may be any amorphous vinyl resin obtained by polymerizing a vinyl compound, and examples thereof include acrylate resins, styrene-acrylate resins, and ethylene-vinyl acetate resin. One of them may be used singly, or two or more thereof may be used in combination. Among them, styrene-acrylate resins (styrene-acrylic resins) are preferred in view of plasticity in heat fixation.

The amorphous vinyl resin preferably has a weight average molecular weight of 20,000 to 150,000 and a number average molecular weight of 5,000 to 20,000 from the viewpoint of achieving fixability and hot offset resistance simultaneously. The weight average molecular weight and the number average molecular weight can be measured in the same manner as in the case of the crystalline resin.

The glass transition temperature of the amorphous vinyl resin is preferably 20 to 70° C. from the viewpoint of achieving fixability and high-temperature storability simultaneously. The glass transition temperature can be measured in accordance with the method defined in ASTM (American Society for Testing Materials standard) D3418-82 (DSC method). For measurement, a DSC-7 differential scanning colorimeter (from PerkinElmer Inc.), a TAC7/DX thermal analysis controller (from PerkinElmer Inc.), etc., can be used.

The amorphous vinyl resin may be a polymer consisting only of a monomer or a copolymer consisting of the mono-

mer and an additional monomer. For the additional monomer, a styrenic monomer such as styrene, a styrene derivative, etc., may be used.

(Amorphous Polyester Resin)

Among polyester resins obtained through polycondensation reaction between a divalent or higher carboxylic acid (polycarboxylic acid) and a dihydric or higher alcohol (polyalcohol), amorphous polyester resins are polyester resins with amorphous characteristics. In the case that a toner having a core-shell structure is formed, an amorphous polyester resin may be used for a material of the shell layer.

For the polycarboxylic acid and the polyalcohol, the materials described above for the crystalline polyester resin may be used.

The ratio between the polycarboxylic acid and the polyalcohol is preferably 1.5/1 to 1/1.5, and more preferably 1.2/1 to 1/1.2 in an equivalent ratio of the hydroxy group of the polyalcohol to the carboxy group of the polycarboxylic acid, [OH]/[COOH].

The number average molecular weight of the amorphous polyester resin is preferably 2,000 to 10,000. The number average molecular weight can be measured in the same manner as in the case of the amorphous vinyl resin.

The glass transition temperature of the amorphous polyester resin is preferably 20 to 70° C. The glass transition temperature can be measured in the same manner as in the case of the amorphous vinyl resin.

The amorphous polyester resin may be, as the above-described crystalline polyester resin, a hybrid amorphous polyester resin modified with a styrene-acrylic resin (hereinafter, also simply referred to as "hybrid amorphous resin").

The styrene-acrylic resin portion has high compatibility with an amorphous vinyl resin and the amorphous polyester resin can be uniformly dispersed in the toner base particle.

In the case that the toner base particle has a core-shell structure and the shell layer contains the amorphous polyester resin, aggregation on the surface of the core particle containing an amorphous vinyl resin tends to occur and the whole surface tends to be covered.

In the present embodiment, "an amorphous polyester resin is modified with a styrene-acrylic resin" refers to a state in which an amorphous polyester resin segment and a styrene-acrylic resin segment chemically bond to each other. An amorphous polyester resin segment refers to a resin portion derived from an amorphous polyester resin, that is, a molecular chain having the same chemical structure as the amorphous polyester resin, in a hybrid resin. A styrene-acrylic resin segment refers to a resin portion derived from a styrene-acrylic resin, that is, a molecular chain having the same chemical structure as the styrene-acrylic resin, in a hybrid resin.

The styrene-acrylic resin can be produced in the same manner by using the materials described above for the hybrid crystalline resin.

The number average molecular weight of the hybrid amorphous polyester resin is preferably 2,000 to 10,000 from the viewpoint of fixability.

The content of the amorphous polyester resin in the toner base particle is preferably 1 to 50 mass % from the viewpoint of fixability and environmental stability of charging.

[Coloring Agent]

For the coloring agent, a known inorganic or organic coloring agent as a coloring agent for a color toner is used. Examples of the coloring agent include carbon black, magnetic materials, pigments, and dyes. One coloring agent or more than one coloring agent may be used.

Examples of the carbon black include channel black, furnace black, acetylene black, thermal black, and lamp

black. Examples of the magnetic material include ferromagnetic metals such as iron, nickel, and cobalt, alloys containing these metals, and compounds of ferromagnetic metals such as ferrite and magnetite.

Examples of the pigment include C. I. Pigment Reds 2, 3, 5, 7, 15, 16, 48:1, 48:3, 53:1, 57:1, 81:4, 122, 123, 139, 144, 149, 166, 177, 178, 208, 209, 222, 238, and 269; C. I. Pigment Oranges 31 and 43; C. I. Pigment Yellows 3, 9, 14, 17, 35, 36, 65, 74, 83, 93, 94, 98, 110, 111, 138, 139, 153, 155, 180, 181, and 185; C. I. Pigment Green 7; C. I. Pigment Blues 15:3, 15:4, and 60; and phthalocyanine pigments whose center metal is zinc, titanium, magnesium, or the like.

Examples of the dye include C. I. Solvent Reds 1, 3, 14, 17, 18, 22, 23, 49, 51, 52, 58, 63, 87, 111, 122, 127, 128, 131, 145, 146, 149, 150, 151, 152, 153, 154, 155, 156, 157, 158, 176, and 179; pyrazolotriazole azo dyes; pyrazolotriazole azomethine dyes; pyrazolone azo dyes; and pyrazolone azomethine dyes; C. I. Solvent Yellows 19, 44, 77, 79, 81, 82, 93, 98, 103, 104, 112, and 162; and C. I. Solvent Blues 25, 36, 60, 70, 93, and 95.

[Release Agent]

Examples of the release agent (wax) include hydrocarbon waxes and ester waxes. Examples of the hydrocarbon wax include low-molecular weight polyethylene wax, low-molecular weight polypropylene wax, Fischer-Tropsch waxes, microcrystalline waxes, and paraffin waxes. Examples of the ester wax include carnauba waxes, pentaerythritol behenate, behenyl behenate, and behenyl citrate. One release agent or more than one release agent may be used.

[Charging-Controlling Agent]

Examples of the charging-controlling agent include nigrosine dyes; metal salts of naphthenic acids or higher fatty acids; alkoxylated amines; quaternary ammonium salt compounds; azo-metal complexes; and metal salicylate and metal complexes thereof. One charging-controlling agent or more than one charging-controlling agent may be used.

[Surfactant]

Examples of the surfactant include anionic surfactants such as sulfate ester salts, sulfonate salts, and phosphate esters; cationic surfactants such as amine salts and quaternary ammonium salts; and nonionic surfactants such as polyethylene glycol-type surfactants, alkylphenol-ethylene oxide adducts, and polyalcohols. One surfactant or more than one surfactant may be used.

Specific examples of the anionic surfactant include sodium dodecylbenzenesulfonate, sodium dodecyl sulfate, sodium alkylphthalenesulfonates, and sodium dialkyl sulfosuccinates. Specific examples of the cationic surfactant include alkylbenzenedimethylammonium chlorides, alkyltrimethylammonium chlorides, and distearylammmonium chloride. Examples of the nonionic surfactant include polyoxyethylene alkyl ethers, glycerin fatty acid esters, sorbitan fatty acid esters, polyoxyethylenesorbitan fatty acid esters, and polyoxyethylene fatty acid esters.

[Structure of Toner Particle]

The structure of the toner particle according to the present embodiment may be a monolayer structure consisting only of the above-described toner particle, or a multilayer structure such as a core-shell structure which includes a core particle of the above-described toner particle and a shell layer covering the core particle and the surface thereof. The shell layer need not cover the whole surface of the core particle, and the core particle may be partially exposed. The cross section of the core-shell structure can be examined, for example, by using known means for observation such as a transmission electron microscope (TEM) and a scanning probe microscope (SPM).

In the case of the core-shell structure, the core particle and the shell layer can be different in properties such as glass transition temperature, melting point, and hardness, and toner particles can be designed in accordance with intended use. For example, a shell layer can be formed by aggregating and fusing a resin having a relatively high glass transition temperature on the surface of the core particle containing a binder resin, a coloring agent, a release agent, etc., and having a relatively low glass transition temperature. As described above, an amorphous polyester resin can be used for the shell layer, and especially, an amorphous polyester resin modified with a styrene-acrylic resin can be preferably used.

[Melting Point]

The toner particle according to the present embodiment preferably has a melting point of 60 to 90° C., and more preferably 65 to 80° C. If the melting point is within the range, sufficient low-temperature fixability and high-temperature storability can be achieved simultaneously. In addition, the thermal resistance (thermal strength) of the toner can be maintained at a satisfactory level, and sufficient high-temperature storability can be obtained. The melting point can be measured in the same manner as the crystalline polyester resin.

[Particle Size of Toner Particle]

The volume-based median diameter of the toner particle according to the present embodiment is preferably 3 to 8  $\mu\text{m}$ , and more preferably 5 to 8  $\mu\text{m}$ . If the volume-based median diameter is within the range, high-resolution dots at approximately 1,200 dpi can be accurately reproduced. The volume-based median diameter can be controlled through the concentration of an aggregating agent used in production, the amount of an organic solvent added, fusion time, the composition of the binder resin, etc.

The volume-based median diameter can be measured by using a measuring apparatus including a Multisizer 3 (from Beckman Coulter, Inc.) to which a computer system with installed data analysis software Software v.3.51 is connected. Specifically, 0.02 g of a sample (toner) is added to 20 mL of a surfactant solution (e.g., a surfactant solution obtained by diluting a neutral detergent containing a surfactant component 10-fold with pure water for the purpose of dispersing a toner particle) and conditioned, and the resultant solution is then subjected to ultrasonic dispersing for 1 minute to prepare a dispersion of a toner. The dispersion of a toner is injected with a pipet into a beaker containing an ISOTON II (from Beckman Coulter, Inc.) in a sample stand until the concentration displayed on the measuring apparatus reaches 8%. This concentration provides a reproducible measurement.

Then, the number of counts for particles to be measured and the aperture diameter for the measuring apparatus are set to 25,000 and 100  $\mu\text{m}$ , respectively, and a measurement range of 2 to 60  $\mu\text{m}$  is divided into 256 portions to calculate a frequency value for each portion, and the particle size at 50% from the largest cumulative volume percentage is determined as the volume-based median diameter.

[Average Circularity of Toner Particle]

In the toner according to the present embodiment, the average circularity of the toner particle is preferably 0.930 to 1.000, and more preferably 0.950 to 0.995. If the average circularity is within the range, the toner particle can be prevented from breaking, and a friction-charging member can be prevented from being stained to stabilize the charging characteristics of the toner. In addition, an image formed with the toner has a high image quality.

The average circularity can be measured as follows. A dispersion of a toner is prepared in the same manner as in the case of the measurement of a median diameter. With an FPIA-2100, an FPIA-3000, (both from Sysmex Corporation, "FPIA" is a registered trademark of this corporation), or the like, an image of the dispersion of a toner is taken in HPF (high-power field) mode with a proper concentration range of 3,000 to 10,000 as HPF detection number, and the circularity of each toner particle is calculated by using equation y. The circularities of the toner particles are added together, and the sum of the circularities is divided by the number of the toner particles to calculate the average circularity. If the HPF detection number is within the proper concentration range, sufficient reproducibility can be obtained. In equation y, L1 represents circumference ( $\mu\text{m}$ ) of a circle having the same projected area as a particle image, and L2 represents perimeter ( $\mu\text{m}$ ) of a projected image of a particle.

$$\text{Circularity} = L1/L2$$

(Equation y)

[External Additive]

The toner particle according to the present embodiment may contain, for example, the toner base particle and an external additive present on the surface of the toner base particle. It is preferable that the toner particle contain an external additive from the viewpoint of controlling flowability, charging characteristics, etc., of the toner particle. One external additive or more than one external additive may be used. Examples of the external additive include a silica particle, a titania particle, an alumina particle, a zirconia particle, a zinc oxide particle, a chromium oxide particle, a cerium oxide particle, an antimony oxide particle, a tungsten oxide particle, a tin oxide particle, a tellurium oxide particle, a manganese oxide particle, and a boron oxide particle.

The external additive preferably contains a silica particle formed through a sol-gel method. Silica particles formed through a sol-gel method have a feature of a narrow particle size distribution, and thus are preferred from the viewpoint of suppressing variation of the attaching strength of the external additive to the toner base particle.

The number average primary particle size of the silica particle is preferably 70 to 200 nm. Silica particles having a number average primary particle size within the range are larger than other external additives. Accordingly, such a silica particle serves as a spacer in a two-component developer, and is preferred from the viewpoint of preventing other smaller external additives from being buried in the toner base particle while a two-component developer is stirred in a developing device. In addition, such a silica particle is preferred also from the viewpoint of preventing the toner base particle from fusing together.

The number average primary particle size of the external additive can be determined, for example, through image processing for an image taken with a transmission electron microscope, and can be adjusted, for example, through classification or mixing with a classified product.

The surface of the external additive preferably has been subjected to hydrophobic treatment. For the hydrophobic treatment, a known surface treating agent is used. One surface treating agent or more than one surface treating agent may be used, and examples thereof include silane coupling agents, silicone oils, titanate coupling agents, aluminate coupling agents, fatty acids, metal salts of fatty acids, esters thereof, and rosin acids.

Examples of the silane coupling agent include dimethyl-dimethoxysilane, hexamethyldisilazane (HMDS), methyltrimethoxysilane, isobutyltrimethoxysilane, and decyl-

rimethoxysilane. Examples of the silicone oil include cyclic compounds and linear or branched organosiloxanes, and more specifically include organosiloxane oligomers, octamethylcyclotetrasiloxane, decamethylcyclotetrasiloxane, tetramethylcyclotetrasiloxane, and tetravinyltetramethylcyclotetrasiloxane.

Examples of the silicone oil include silicone oils which are highly reactive and at least one end of which is modified by introducing a modifying group to a side chain, one end, both ends, one end of a side chain, both ends of a side chain, or the like. One type of a modifying group or more than one type of modifying groups may be used, and examples of the modifying group include an alkoxy group, a carboxyl group, a carbinol group, a higher fatty acid modifying group, a phenol group, an epoxy group, a methacryl group, and an amino group.

The amount of the external additive to be added is preferably 0.1 to 10.0 mass %, and more preferably 1.0 to 3.0 mass % based on the total amount of the toner particle.

[Developer]

The toner is composed of the toner particle itself in the case of a one-component developer, and composed of the toner particle and a carrier particle in the case of a two-component developer. The content of the toner particle (toner concentration) in the two-component developer may be the same as that in common two-component developers, and for example, is 4.0 to 8.0 mass %.

The carrier particle is composed of a magnetic material. Examples of the carrier particle include a coated carrier particle including a core material particle consisting of the magnetic material and a coating layer covering the surface of the core material particle, and a resin-dispersed carrier particle including a fine particle of a magnetic material dispersed in a resin. The carrier particle is preferably the coated carrier particle from the viewpoint of preventing the carrier particle from attaching to a photoconductor.

The core material particle is composed of a magnetic material such as a substance which is strongly magnetized by a magnetic field in the direction of the magnetic field. One magnetic material or more than one magnetic material may be used, and examples thereof include ferromagnetic metals such as iron, nickel, and cobalt; alloys or compounds containing these metals; and alloys which exhibit ferromagnetism via heat treatment.

Examples of the ferromagnetic metal and compound containing it include iron, ferrites represented by formula (a), and magnetites represented by formula (b). M in formula (a) and formula (b) denotes one or more monovalent or divalent metals selected from the group consisting of Mn, Fe, Ni, Co, Cu, Mg, Zn, Cd, and Li.



Formula (a)



Formula (b)

Examples of the alloy or metal oxide which exhibits ferromagnetism via heat treatment include Heusler alloys such as manganese-copper-aluminum and manganese-copper-tin; and chromium dioxide.

The core material particle is preferably the ferrite. The reason is that impact force due to stirring in a developing device can be reduced because the specific gravity of the coated carrier particle is smaller than that of a metal constituting the core material particle.

One coating material or more than one coating material may be used. For the coating material, a known resin for covering a core material particle of a carrier particle may be used. The coating material is preferably a resin having a

cycloalkyl group from the viewpoint of the lowering of the moisture adsorption of the carrier particle and the enhancement of the adhesion of the coating layer to the core material particle. Examples of the cycloalkyl group include a cyclohexyl group, a cyclopentyl group, a cyclopropyl group, a cyclobutyl group, a cycloheptyl group, a cyclooctyl group, a cyclononyl group, and a cyclodecyl group. Among them, a cyclohexyl group and a cyclopentyl group are preferred, and a cyclohexyl group is more preferred from the viewpoint of the adhesion of the coating layer to a ferrite particle.

The weight average molecular weight of the resin having a cycloalkyl group is, for example, 10,000 to 800,000, and more preferably 100,000 to 750,000. The content of the cycloalkyl group in the resin is, for example, 10 to 90 mass %. The content of the cycloalkyl group in the resin can be determined by using a known instrumental analysis method such as pyrolysis-gas chromatography/mass spectrometry (Py-GC/MS) and proton magnetic resonance spectroscopy (<sup>1</sup>H-NMR).

The two-component developer can be produced by mixing the toner particle and the carrier particle in appropriate amounts. Examples of mixing apparatuses for the mixing include a Nauta mixer, and W-cone and V-shaped mixers.

The size and shape of the toner particle may be appropriately determined as long as the advantageous effects of the present embodiment can be obtained. For example, the volume average particle size of the toner particle is 3.0 to 8.0  $\mu\text{m}$ , and the average circularity of the toner particle is 0.920 to 1.000.

Similarly, the size and shape of the carrier particle may be appropriately determined as long as the advantageous effects of the present embodiment can be obtained. The volume average particle size of the carrier particle is, for example, 15 to 100  $\mu\text{m}$ . The volume average particle size of the carrier particle can be measured, for example, by using a wet method with the laser diffraction particle size distribution measuring apparatus "HELOS KA" (from Japan Laser Corporation). The volume average particle size of the carrier particle can be adjusted, for example, through a method of controlling the particle size of the core material particle via production conditions for the core material particle, classification of the carrier particle, or mixing with a classified product of a carrier particle.

As described above, the process for producing a toner according to the present embodiment includes: a first step of heating a dispersion containing an aqueous medium and a binder resin containing a crystalline resin to a temperature higher than or equal to a melting point of the crystalline resin in a production step for forming a toner base particle by aggregating and fusing a fine particle of the binder resin containing the crystalline resin in the presence of a metal ion; and a second step of maintaining the dispersion at temperature T (°C.) for 30 minutes or longer in a state where a pH of the dispersion is maintained at 5.5 or higher and 9.0 or lower, in which the temperature T satisfies the following expression,  $Rc-25 \leq T \leq Rc-5$ , where the Rc represents a recrystallization temperature (°C.) of the crystalline resin.

One of the features of the above process for producing a toner is that a toner having excellent low-temperature fixability and low density unevenness of images to be formed can be obtained, and the reason is presumably as follows.

As described above, in the present embodiment a toner base particle is produced by an emulsion aggregation method in which fine particles of a binder resin is aggregated in the presence of a metal ion as an aggregating agent. Because a dispersion containing the toner base particle is subjected to heat treatment under a particular heat treatment

scheme, domains of a crystalline resin are deemed to be finely dispersed in the toner base particle without being present in the vicinity of the surface of the toner base particle. In addition, because a pH of the dispersion is maintained at 5.5 or higher during the heat treatment, an acid group of the binder resin does not dissociate. Accordingly, a crosslinking amount by the metal ion, which aggregates the fine particles of the binder resin, is not lowered, and as a result increase in a domain diameter of the crystalline resin and/or bleeding of the crystalline resin into the vicinity of the surface of the toner base particle is presumably suppressed. Further, since the pH of the dispersion is maintained at 9.0 or lower during the heat treatment, it is considered that the crosslinking amount by the metal ion does not increase excessively and the fine particles of the binder resin do not aggregate too tightly, resulting in suppressed deterioration of low-temperature fixability.

Thus, in a toner produced by the production process of the present embodiment, a domain diameter of a crystalline resin does not increase and a finely dispersed state of the crystalline resin domains in the toner base particle is maintained. Accordingly, deterioration of surface resistance, charging characteristics, and so forth of a toner are presumably suppressed, achieving low-temperature fixability of a toner and suppressed density unevenness of images.

T satisfying  $Rc-25 \leq T \leq Rc-5$  is more effective from the viewpoint of enhancing low-temperature fixability of a toner and suppressing density unevenness of images.

Further including a step of cooling the dispersion having been heated to a temperature higher than Rc to a temperature lower than  $Rc-25$  °C. is more effective from the viewpoint of suppressing density unevenness of images.

Further including a step of cooling the dispersion having been heated to a temperature higher than Rc to a temperature lower than Rc at a temperature-lowering rate of 1 °C./min or higher is more effective from the viewpoint of enhancing low-temperature fixability.

The use of a crystalline polyester resin as the crystalline resin is more effective from the viewpoint of enhancing low-temperature fixability.

The toner is applied to common electrophotographic image forming methods, and is used for development of electrostatic latent images.

As evident from the above description, a process for producing a toner according to the present embodiment can accurately control a presence state and a domain diameter of a crystalline resin in a toner even during heat treatment, and consequently both low-temperature fixability and suppressed density unevenness of images can be achieved.

## EXAMPLES

Hereinafter, the present invention will be described more specifically with reference to Examples and Comparative Examples, but the present invention is never limited to Examples below.

[Synthesis of Crystalline Polyester Resin and Preparation of Dispersion Thereof]

(Synthesis of Crystalline Polyester Resin 1)

The following raw material monomers of an addition polymerization resin (styrene-acrylic resin: StAc) segment, including bireactive monomers, and radical polymerization initiator were placed in a dropping funnel.

|                                                   |                      |
|---------------------------------------------------|----------------------|
| Styrene                                           | 36.0 parts by weight |
| n-Butyl acrylate                                  | 13.0 parts by weight |
| Acrylic acid                                      | 2.0 parts by weight  |
| Polymerization initiator<br>(di-t-butyl peroxide) | 7.0 parts by weight  |

The following raw material monomers of a polycondensation resin (crystalline polyester resin: CPEs) segment were placed in a four-necked flask equipped with a nitrogen inlet tube, a dehydration tube, a stirrer, and a thermocouple, and heated to 170° C. to dissolve.

|                       |                     |
|-----------------------|---------------------|
| Tetradecanedioic acid | 440 parts by weight |
| 1,4-Butanediol        | 153 parts by weight |

Subsequently, the raw materials of an addition polymerization resin (StAc) were added dropwise to the dissolved monomer solution under stirring over 90 minutes, and the resultant solution was aged for 60 minutes and then unreacted addition-polymerizable monomers were removed under reduced pressure (8 kPa). The amount of the removed monomers was only a trace amount relative to the raw material monomer of the resin. Thereafter, 0.8 part by weight of Ti(OBu)<sub>4</sub> as an esterification catalyst was added thereto, and the temperature was elevated to 235° C., and reaction was performed under atmospheric pressure (101.3 kPa) for 5 hours and then under reduced pressure (8 kPa) for 1 hour.

The resultant mixture was then cooled to 200° C. and subsequently allowed to react under reduced pressure (20 kPa) for 1 hour to afford crystalline polyester resin 1. The weight average molecular weight, melting point, and recrystallization temperature (Rc) of crystalline polyester resin 1 obtained were 24,500, 75.5° C., and 70.6° C., respectively.

(Preparation of Crystalline Polyester Resin Particle Dispersion 1)

Crystalline polyester resin 1 in an amount of 100 parts by weight was dissolved in 400 parts by weight of ethyl acetate (from KANTO CHEMICAL CO., INC.), and the resultant solution was mixed with 638 parts by weight of a 0.26 mass % sodium lauryl sulfate solution prepared in advance. The resultant mixed solution was subjected to ultrasonic dispersing with the ultrasonic homogenizer US-150T (from NISSEI Corporation) at 300 μA of V-LEVEL under stirring for 30 minutes. Thereafter, the resultant dispersion was warmed to 40° C., and at the temperature the ethyl acetate was completely removed with the diaphragm vacuum pump V-700 (from BUCHI Ladotechnik AG) under reduced pressure and stirring for 3 hours to prepare crystalline polyester resin particle dispersion 1. The crystalline polyester resin particle in the dispersion had a volume-based median diameter of 160 nm.

(Synthesis of Crystalline Polyester Resin 2)

In a reaction vessel equipped with a stirrer, a thermometer, a condenser, and a nitrogen inlet tube, 315 parts by weight of tetradecanedioic acid and 252 parts by weight of 1,4-butanediol were placed. The inside of the reaction vessel was purged with dry nitrogen gas, and then 0.1 part by weight of titanium tetrabutoxide was added thereto, and polymerization reaction was performed under stirring in a nitrogen gas flow at 180° C. for 8 hours. Further, 0.2 part by weight of titanium tetrabutoxide was added thereto, and the temperature was elevated to 220° C., and polymerization reaction was performed under stirring for 6 hours. Thereafter, the pressure in the reaction vessel was reduced to 10

mmHg (13.3 hPa), and reaction was performed under reduced pressure to obtain crystalline polyester resin 2. The weight average molecular weight, melting point, and recrystallization temperature (Rc) of crystalline polyester resin 2 obtained were 22,000, 75.0° C., and 70.8° C., respectively.

(Preparation of Crystalline Polyester Resin Particle Dispersion 2)

Crystalline polyester resin 2 in an amount of 100 parts by weight was dissolved in 400 parts by weight of ethyl acetate (from KANTO CHEMICAL CO., INC.), and the resultant solution was mixed with 638 parts by weight of a 0.26 mass % sodium lauryl sulfate solution prepared in advance. The mixed solution was subjected to ultrasonic dispersing with the ultrasonic homogenizer US-150T (from NISSEI Corporation) at 300 μA of V-LEVEL under stirring for 30 minutes. Thereafter, the resultant dispersion was warmed to 40° C., and at the temperature the ethyl acetate was completely removed with the diaphragm vacuum pump V-700 (from BUCHI Ladotechnik AG) under reduced pressure and stirring for 3 hours to prepare crystalline polyester resin particle dispersion 2. The crystalline polyester resin particle in the dispersion had a volume-based median diameter of 160 nm.

(Synthesis of Crystalline Polyester Resin 3)

In a reaction vessel equipped with a stirring apparatus, a nitrogen inlet tube, a temperature sensor, and a rectifying column, 200 parts by weight of dodecanedioic acid and 102 parts by weight of 1,6-hexanediol were fed, and the temperature of the reaction system was elevated to 190° C. over 1 hour. After confirmation that the reaction system was uniformly stirred, 0.3 part by weight of Ti(OBu)<sub>4</sub> as a catalyst was added thereto and the temperature of the reaction system was further elevated from 190° C. to 240° C. over 6 hours while evaporating and removing generated water, and dehydration condensation reaction was continuously performed for 6 hours with the temperature maintained at 240° C. for polymerization to obtain crystalline polyester resin 3. The weight average molecular weight, melting point, and recrystallization temperature (Rc) of crystalline polyester resin 3 obtained were 14,500, 70° C., and 65.8° C., respectively.

(Preparation of Crystalline Polyester Resin Particle Dispersion 3)

Crystalline polyester resin 3 in an amount of 100 parts by weight was dissolved in 400 parts by weight of ethyl acetate (from KANTO CHEMICAL CO., INC.), and the resultant solution was mixed with 638 parts by weight of a 0.26 mass % sodium lauryl sulfate solution prepared in advance. The mixed solution was subjected to ultrasonic dispersing with the ultrasonic homogenizer US-150T (from NISSEI Corporation) at 300 μA of V-LEVEL under stirring for 30 minutes. Thereafter, the resultant dispersion was warmed to 40° C., and at the temperature the ethyl acetate was completely removed with the diaphragm vacuum pump V-700 (from BUCHI Ladotechnik AG) under reduced pressure and stirring for 3 hours to prepare crystalline polyester resin particle dispersion 3. The crystalline polyester resin particle in the dispersion had a volume-based median diameter of 160 nm.

(Preparation of Coloring Agent Particle Dispersion)

To a solution prepared by adding 90 parts by weight of sodium dodecyl sulfate to 1,600 parts by weight of deionized water, 420 parts by weight of copper phthalocyanine (C. I. Pigment Blue 15:3) was gradually added under stirring. The resultant solution was dispersed with the stirring apparatus CLEARMIX (from M Technique Co., Ltd., "CLEARMIX" is a registered trade name) to prepare a coloring agent particle dispersion. The coloring agent particle in the dispersion had a volume-based median diameter of 110 nm.

[Preparation of Amorphous Vinyl Resin Particle Dispersion for Core]

(First Stage of Polymerization)

In a 5 L reaction vessel equipped with a stirring apparatus, a temperature sensor, a condenser, and a nitrogen inlet tube, 8 parts by weight of sodium dodecyl sulfate and 3,000 parts by weight of deionized water were fed, and the internal temperature was elevated to 80° C. under stirring at a stirring rate of 230 rpm in a nitrogen gas flow. After the temperature elevation, a solution prepared by dissolving 10 parts by weight of potassium persulfate in 200 parts by weight of deionized water was added thereto, and the temperature of the solution was again set to 80° C. and a mixed solution of the following monomers was added dropwise thereto over 1 hour.

|                  |                       |
|------------------|-----------------------|
| Styrene          | 480.0 parts by weight |
| n-Butyl acrylate | 250.0 parts by weight |
| Methacrylic acid | 68.0 parts by weight  |

After the dropwise addition of the mixed solution, the resultant solution was heated and stirred at 80° C. for 2 hours to polymerize the monomers, and thus an amorphous vinyl resin particle dispersion for a core was prepared.

(Second Stage of Polymerization)

In a 5 L reaction vessel equipped with a stirring apparatus, a temperature sensor, a condenser, and a nitrogen inlet tube, a solution prepared by dissolving 7 parts by weight of sodium polyoxyethylene (2) dodecyl ether sulfate in 3,000 parts by weight of deionized water was fed, and heated to 98° C. After the heating, the amorphous vinyl resin particle dispersion prepared in the first stage of polymerization in an amount of 80 parts by weight in terms of solids content, and a mixed solution prepared by dissolving the following monomers, chain transfer agent, and release agent at 90° C. were added thereto.

|                                                         |                       |
|---------------------------------------------------------|-----------------------|
| Styrene (St)                                            | 285.0 parts by weight |
| n-Butyl acrylate (BA)                                   | 95.0 parts by weight  |
| Methacrylic acid (MAA)                                  | 20.0 parts by weight  |
| n-Octyl 3-mercaptopropionate (chain transfer agent)     | 1.5 parts by weight   |
| Behenyl behenate (release agent, melting point: 73° C.) | 190.0 parts by weight |

Mixing and dispersing was carried out with a CLEAR-MIX (from M Technique Co., Ltd.), a mechanical disperser having a circulation path, for 1 hour to prepare a dispersion containing an emulsified particle (oil droplet). To this dispersion, a solution of a polymerization initiator prepared by dissolving 6 parts by weight of potassium persulfate in 200 parts by weight of deionized water was added, and this system was heated and stirred at 84° C. over 1 hour for polymerization to prepare an amorphous vinyl resin particle dispersion.

(Third Stage of Polymerization)

To the amorphous vinyl resin particle dispersion obtained in the second stage of polymerization, 400 parts by weight of deionized water was further added and thoroughly mixed, and then a solution prepared by dissolving 11 parts by weight of potassium persulfate in 400 parts by weight of deionized water was added thereto. Furthermore, a mixed solution of the following monomers and chain transfer agent was added dropwise thereto under a temperature condition of 82° C. over 1 hour.

|                              |                       |
|------------------------------|-----------------------|
| Styrene (St)                 | 454.8 parts by weight |
| 2-Ethylhexyl acrylate (2EHA) | 143.2 parts by weight |
| Methacrylic acid (MAA)       | 52.0 parts by weight  |
| n-Octyl 3-mercaptopropionate | 8.0 parts by weight   |

After the dropwise addition, the resultant solution was heated and stirred over 2 hours for polymerization, and then cooled to 28° C. to prepare an amorphous vinyl resin dispersion for a core.

[Amorphous Polyester Resin for Shell Layer]

A mixed solution of the following monomers of a styrene-acrylic resin, monomer having a substituent capable of reacting with both of an amorphous polyester resin and the styrene-acrylic resin, and polymerization initiator was placed in a dropping funnel.

|                                                |                      |
|------------------------------------------------|----------------------|
| Styrene                                        | 80.0 parts by weight |
| n-Butyl acrylate                               | 20.0 parts by weight |
| Acrylic acid                                   | 10.0 parts by weight |
| Di-t-butyl peroxide (polymerization initiator) | 16.0 parts by weight |

The following monomers of an amorphous polyester resin were placed in a four-necked flask equipped with a nitrogen inlet tube, a dehydration tube, a stirrer, and a thermocouple, and heated to 170° C. to dissolve.

|                                            |                       |
|--------------------------------------------|-----------------------|
| Bisphenol A - propylene oxide adduct (1:2) | 285.7 parts by weight |
| Terephthalic acid                          | 66.9 parts by weight  |
| Fumaric acid                               | 47.4 parts by weight  |

The mixed solution placed in the dropping funnel was added dropwise into the four-necked flask over 90 minutes under stirring, and the resultant solution was aged for 60 minutes, and unreacted monomers were then removed under reduced pressure (8 kPa). Thereafter, 0.4 part by weight of Ti(OBu)<sub>4</sub> as an esterification catalyst was added thereto, and the temperature was elevated to 235° C., and reaction was performed under atmospheric pressure (101.3 kPa) for 5 hours and then under reduced pressure (8 kPa) for 1 hour. The resultant solution was then cooled to 200° C. and allowed to react under reduced pressure (20 kPa) for 1 hour, and subsequently the solvent was removed to afford an amorphous polyester resin for a shell layer modified with a styrene-acrylic resin. The weight average molecular weight and the glass transition temperature of the amorphous polyester resin for a shell layer obtained were 25,000 and 60° C., respectively. The weight average molecular weight was measured in the same manner as in the case of the above-described crystalline polyester resin, and the glass transition temperature was measured in the same manner as in the case of the amorphous vinyl resin.

[Preparation of Amorphous Polyester Resin Particle Dispersion for Shell Layer]

The amorphous polyester resin for a shell layer in an amount of 100 parts by weight was dissolved in 400 parts by weight of ethyl acetate (from KANTO CHEMICAL CO., INC.), and the resultant solution was mixed with 638 parts by weight of a 0.26 mass % sodium lauryl sulfate solution prepared in advance. The mixed solution was subjected to ultrasonic dispersing with the ultrasonic homogenizer US-150T (from NISSEI Corporation) at 300 μA of V-LEVEL under stirring for 30 minutes. Thereafter, the resultant dispersion was warmed to 40° C., and at the

25

temperature the ethyl acetate was completely removed with the diaphragm vacuum pump V-700 (from BUCHI Ladotechnik AG) under reduced pressure and stirring for 3 hours to prepare an amorphous polyester resin particle dispersion for a shell layer having a solids content of 13.5 mass %. The amorphous polyester resin particle in the dispersion had a volume-based median diameter of 160 nm.

## Example 1: Production of Toner 1

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060  
9065  
9070  
9075  
9080  
9085  
9090  
9095  
9100  
9105  
9110  
9115  
9120  
9125  
9130  
9135  
9140  
9145  
9150  
9155  
9160  
9165  
9170  
9175  
9180  
9185  
9190  
9195  
9200  
9205  
9210  
9215  
9220  
9225  
9230  
9235  
9240  
9245  
9250  
9255  
9260  
9265  
9270  
9275  
9280  
9285  
9290  
9295  
9300  
9305  
9310  
9315  
9320  
9325  
9330  
9335  
9340  
9345  
9350  
9355  
9360  
9365  
9370  
9375  
9380  
9385  
9390  
9395  
9400  
9405  
9410  
9415  
9420  
9425  
9430  
9435  
9440  
9445  
9450  
9455  
9460<br

## Examples 14 to 16: Production of Toners 14 to 16

Toners 14 to 16 were produced in the same manner as in Example 1 except that the heat treatment step was changed to schemes 7 to 9 listed in Table 1, respectively, and the cooling rate at Rc was changed to 2° C./min.

## Example 17: Production of Toner 17

Toner 17 was produced in the same manner as in Example 1 except that the heat treatment step was changed to scheme 6 listed in Table 1, the cooling rate at Rc was changed to 2° C./min, and crystalline resin 1 was changed to crystalline resin 2.

## Example 18: Production of Toner 18

Toner 18 was produced in the same manner as in Example 1 except that the heat treatment step was changed to scheme 10 listed in Table 1, the cooling rate at Rc was changed to 2° C./min, and crystalline resin 1 was changed to crystalline resin 2.

## Example 19: Production of Toner 19

Toner 19 was produced in the same manner as in Example 1 except that the heat treatment step was changed to scheme 11 listed in Table 1, the cooling rate at Rc was changed to 2° C./min, and crystalline resin 1 was changed to crystalline resin 3.

## Example 20: Production of Toner 20

Toner 20 was produced in the same manner as in Example 1 except that the heat treatment step was changed to scheme 12 listed in Table 1, the cooling rate at Rc was changed to 2° C./min, and crystalline resin 1 was changed to crystalline resin 3.

## Comparative Example 1: Production of Toner 21

Toner 21 was produced in the same manner as in Example 1 except that the heat treatment step was changed to scheme 6 listed in Table 1, the cooling rate at Rc was changed to 2° C./min, and the pH of the dispersion in the heat treatment step was changed to 10.0.

## Comparative Example 2: Production of Toner 22

Toner 22 was produced in the same manner as in Comparative Example 1 except that the pH of the dispersion in the heat treatment step was changed to 4.0.

## Comparative Example 3: Production of Toner 23

Toner 23 was produced in the same manner as in Example 1 except that the heat treatment step was changed to scheme 13 listed in Table 1 and the cooling rate at Rc was changed to 2° C./min.

## Comparative Example 4: Production of Toner 24

Toner 24 was produced in the same manner as in Comparative Example 3 except that the heat treatment step was changed to scheme 14 listed in Table 1.

## Comparative Example 5: Production of Toner 25

In the process for producing toner 1, a dispersion of a toner base particle was cooled without being subjected to a

heat treatment step. Solid-liquid separation was then performed, and the dehydrated toner cake was dispersed in deionized water again, and washed through three cycles of solid-liquid separation, and dried at 40° C. for 24 hours. The toner base particle obtained was left to stand in an environment of 60° C. and 50% RH for 60 minutes. To 100 parts by weight of the toner base particle obtained, 0.6 part by weight of a hydrophobic silica particle (number average primary particle size: 12 nm, degree of hydrophobicity: 68), 1.0 part by weight of a hydrophobic titanium oxide particle (number average primary particle size: 20 nm, degree of hydrophobicity: 63), and 1.0 part by weight of sol-gel silica (number average primary particle size=110 nm) were added, and the resultant composition was mixed by using a Henschel mixer (from NIPPON COKE & ENGINEERING Co., LTD.) with a peripheral speed of the rotating blade of 35 mm/sec at 32° C. for 20 minutes. After mixing, coarse particles were removed with a sieve having a mesh size of 45 µm to obtain toner 25.

## Comparative Example 6: Production of Toner 26

|                                                         |                      |
|---------------------------------------------------------|----------------------|
| Styrene (St)                                            | 50.0 parts by weight |
| n-Butyl acrylate (BA)                                   | 16.7 parts by weight |
| Methacrylic acid (MAA)                                  | 3.5 parts by weight  |
| Behenyl behenate (release agent, melting point: 73° C.) | 7.0 parts by weight  |
| Crystalline polyester resin 1                           | 8.0 parts by weight  |

The above raw materials were mixed together, and a 15 mm ceramic bead was added thereto, and the resultant mixture was dispersed with an attritor (from NIPPON COKE & ENGINEERING Co., LTD.) for 2 hours to obtain a polymerizable monomer composition. Subsequently, 800 parts of deionized water and 15.5 parts of tricalcium phosphate were added into a container equipped with the high-speed stirring apparatus TK-homomixer (from Tokushu Kika Kogyo Co., Ltd.), and the rotational speed was adjusted to 15,000 rpm and the temperature was elevated to 70° C. to obtain an aqueous dispersion medium. To the above polymerizable monomer composition, 4.0 parts of t-butyl peroxypivalate as a polymerization initiator was added, and the resultant composition was added to the aqueous dispersion medium. Dispersing was performed for granulation by using the high-speed stirring apparatus for 3 minutes, with the rotational speed maintained at 15,000 rpm. Thereafter, the high-speed stirring apparatus was replaced with a stirring apparatus having a propeller stirring blade, and polymerization was performed under stirring at 150 rpm for 8.0 hours with the temperature maintained at 70° C., and the temperature was elevated to 80° C. and heating was performed for 4 hours. Heat treatment was then performed by using the same scheme for toner 7.

Subsequently, solid-liquid separation was performed, and the dehydrated toner cake was dispersed in deionized water again, and washed through three cycles of solid-liquid separation. After washing, the resultant toner cake was dried at 40° C. for 24 hours to afford a toner particle. To 100 parts by weight of the toner particle obtained, 0.6 part by weight of a hydrophobic silica particle (number average primary particle size: 12 nm, degree of hydrophobicity: 68), 1.0 part by weight of a hydrophobic titanium oxide particle (number average primary particle size: 20 nm, degree of hydrophobicity: 63), and 1.0 part by weight of sol-gel silica (number average primary particle size=110 nm) were added, and the

resultant composition was mixed by using a Henschel mixer (from NIPPON COKE & ENGINEERING Co., LTD.) with a peripheral speed of a rotating blade of 35 mm/sec at 32° C. for 20 minutes. After mixing, coarse particles were removed with a sieve having a mesh size of 45 µm to obtain toner 26.

Table 1 shows heat treatment schemes for toners. In Table 1 below, “ $T_0$ ” denotes a pre-heat treatment step temperature, “ $T_s$ ” denotes an initiation temperature of the heat treatment step, and “ $T_E$ ” denotes a termination temperature of the heat treatment step.

TABLE 1

| Scheme<br>(No.) | Heat treatment step |                 |                 |           |                   |
|-----------------|---------------------|-----------------|-----------------|-----------|-------------------|
|                 | $T_0$<br>(° C.)     | $T_s$<br>(° C.) | $T_E$<br>(° C.) | Scheme    | Duration<br>(min) |
| 1               | 65                  | 65              | 61              | cooling   | 30                |
| 2               | 65                  | 65              | 61              | cooling   | 60                |
| 3               | 60                  | 65              | 65              | retention | 60                |
| 4               | 60                  | 60              | 60              | retention | 60                |
| 5               | 45                  | 60              | 60              | retention | 60                |
| 6               | 30                  | 60              | 60              | retention | 60                |
| 7               | 30                  | 55              | 55              | retention | 60                |
| 8               | 30                  | 50              | 50              | retention | 60                |
| 9               | 30                  | 46              | 46              | retention | 60                |
| 10              | 30                  | 60              | 60              | retention | 120               |
| 11              | 30                  | 55              | 55              | retention | 60                |
| 12              | 30                  | 41              | 41              | retention | 60                |
| 13              | 30                  | 70              | 70              | retention | 60                |
| 14              | 30                  | 67              | 67              | retention | 60                |

[Evaluation for Toners]

(Evaluation on Low-Temperature Fixability (Under-Off-set)]

The term “under-offset” refers to an image defect in which a toner peels off from a transfer material such as a recording sheet because melting of a toner layer by heat provided in passing through a fixing apparatus is insufficient. For evaluation on low-temperature fixability, each toner produced in the above was sequentially loaded on an image forming

apparatus and an unfixed solid image (attached amount 11.3 g/m<sup>2</sup>) was formed on mondi Color Copy (A4, 90 g/m<sup>2</sup>; from Mondi plc) with the image forming apparatus in an environment of room temperature and normal humidity (20° C., 50% RH). Subsequently, the surface temperature of a pressure roller of the fixing apparatus was set to 100° C. and the images were fixed with the surface temperature of a heating roller changed at an interval of 2° C. within the range of 130 to 170° C. Then, the lower limit temperature for fixing (Tf) without under-offset was measured for the upper fixing belt.

Using the following evaluation criteria, low-temperature fixability was evaluated, and lower than 150° C. of a lower limit temperature for fixing was regarded as being acceptable. The results are shown in Tables 2 and 3.

(Density Unevenness of Images)

In an environment of room temperature and normal humidity (20° C., 55% RH), whole-surface solid images with original image density 1.30 were formed on 100 sheets of A4 wood-free paper (64 g/m<sup>2</sup>). Then, an original with a set solid image having original reflection densities 1.30 at total five points of the four corners and the central part of the image was duplicated, and relative reflection densities of the output images based on white paper were measured at the five points. The difference  $\Delta G$  between the maximum and minimum values of the image reflection densities measured as above at the five points was interpreted as density unevenness of images. Lower than 0.10 of density unevenness of images was regarded as being acceptable. The results are shown in Tables 2 and 3.

In Tables 2 and 3, “NPC” denotes an emulsion polymerization aggregation method (emulsion aggregation method), “SP” denotes a suspension polymerization method, “Tm” denotes a melting point of a crystalline resin, “temperature” of a dispersion indicates a temperature of the dispersion in the first step, “cooling rate” indicates a cooling rate in passing through Rc, “pH” indicates a pH of a dispersion at a pre-heat treatment temperature, “scheme” indicates a scheme for heat treatment, and “Tf” denotes a lower limit temperature for fixing.

TABLE 2

| Example | Toner | Production | Crystalline |      |         |     | Dispersion   |              |                       |                            | pH  | Scheme | Tf | $\Delta G$ |
|---------|-------|------------|-------------|------|---------|-----|--------------|--------------|-----------------------|----------------------------|-----|--------|----|------------|
|         |       |            | No.         | No.  | process | No. | Tm<br>(° C.) | Rc<br>(° C.) | Temperature<br>(° C.) | Cooling rate<br>(° C./min) |     |        |    |            |
| 1       | 1     | NPC        | 1           | 75.5 | 70.6    | 80  | 1            | aqueous      | 7                     | 1                          | 144 | 0.09   |    |            |
| 2       | 2     | NPC        | 1           | 75.5 | 70.6    | 80  | 1            | aqueous      | 7                     | 2                          | 144 | 0.09   |    |            |
| 3       | 3     | NPC        | 1           | 75.5 | 70.6    | 80  | 1            | aqueous      | 7                     | 3                          | 144 | 0.08   |    |            |
| 4       | 4     | NPC        | 1           | 75.5 | 70.6    | 80  | 1            | aqueous      | 7                     | 4                          | 140 | 0.07   |    |            |
| 5       | 5     | NPC        | 1           | 75.5 | 70.6    | 80  | 1            | aqueous      | 7                     | 5                          | 140 | 0.06   |    |            |
| 6       | 6     | NPC        | 1           | 75.5 | 70.6    | 80  | 1            | aqueous      | 7                     | 6                          | 140 | 0.05   |    |            |
| 7       | 7     | NPC        | 1           | 75.5 | 70.6    | 80  | 2            | aqueous      | 7                     | 6                          | 138 | 0.03   |    |            |
| 8       | 8     | NPC        | 1           | 75.5 | 70.6    | 80  | 5            | aqueous      | 7                     | 6                          | 136 | 0.01   |    |            |
| 9       | 9     | NPC        | 1           | 75.5 | 70.6    | 80  | 0.5          | aqueous      | 7                     | 6                          | 142 | 0.07   |    |            |
| 10      | 10    | NPC        | 1           | 75.5 | 70.6    | 80  | 2            | aqueous      | 8                     | 6                          | 136 | 0.02   |    |            |
| 11      | 11    | NPC        | 1           | 75.5 | 70.6    | 80  | 2            | aqueous      | 9                     | 6                          | 144 | 0.01   |    |            |
| 12      | 12    | NPC        | 1           | 75.5 | 70.6    | 80  | 2            | aqueous      | 6                     | 6                          | 136 | 0.04   |    |            |
| 13      | 13    | NPC        | 1           | 75.5 | 70.6    | 80  | 2            | aqueous      | 5.5                   | 6                          | 134 | 0.06   |    |            |
| 14      | 14    | NPC        | 1           | 75.5 | 70.6    | 80  | 2            | aqueous      | 7                     | 7                          | 138 | 0.03   |    |            |
| 15      | 15    | NPC        | 1           | 75.5 | 70.6    | 80  | 2            | aqueous      | 7                     | 8                          | 136 | 0.03   |    |            |

TABLE 3

| No.         | Toner No. | Production process | Crystalline resin |          | Dispersion        |                        |         |        |            |          |        |
|-------------|-----------|--------------------|-------------------|----------|-------------------|------------------------|---------|--------|------------|----------|--------|
|             |           |                    | Tm No. (°C.)      | Rc (°C.) | Temperature (°C.) | Cooling rate (°C./min) | Medium  | pH (-) | Scheme No. | Tf (°C.) | ΔG (-) |
| Example 16  | 16        | NPC                | 1 75.5            | 70.6     | 80                | 2                      | aqueous | 7      | 9          | 134      | 0.04   |
| Example 17  | 17        | NPC                | 2 75.0            | 70.8     | 80                | 2                      | aqueous | 7      | 6          | 136      | 0.03   |
| Example 18  | 18        | NPC                | 2 75.0            | 70.8     | 80                | 2                      | aqueous | 7      | 10         | 136      | 0.02   |
| Example 19  | 19        | NPC                | 3 70.0            | 65.8     | 80                | 2                      | aqueous | 7      | 11         | 134      | 0.04   |
| Example 20  | 20        | NPC                | 3 70.0            | 65.8     | 80                | 2                      | aqueous | 7      | 12         | 134      | 0.06   |
| Comparative | 21        | NPC                | 1 75.5            | 70.6     | 80                | 2                      | aqueous | 10     | 6          | 154      | 0.01   |
| Example 1   |           |                    |                   |          |                   |                        |         |        |            |          |        |
| Comparative | 22        | NPC                | 1 75.5            | 70.6     | 80                | 2                      | aqueous | 4      | 6          | 134      | 0.10   |
| Example 2   |           |                    |                   |          |                   |                        |         |        |            |          |        |
| Comparative | 23        | NPC                | 1 75.5            | 70.6     | 80                | 2                      | aqueous | 7      | 13         | 156      | 0.15   |
| Example 3   |           |                    |                   |          |                   |                        |         |        |            |          |        |
| Comparative | 24        | NPC                | 1 75.5            | 70.6     | 80                | 2                      | aqueous | 7      | 14         | 154      | 0.09   |
| Example 4   |           |                    |                   |          |                   |                        |         |        |            |          |        |
| Comparative | 25        | NPC                | 1 75.5            | 70.6     | 80                | 2                      | —       | —      | —          | 156      | 0.15   |
| Example 5   |           |                    |                   |          |                   |                        |         |        |            |          |        |
| Comparative | 26        | SP                 | 1 75.5            | 70.6     | 80                | 2                      | aqueous | 7      | 6          | 150      | 0.15   |
| Example 6   |           |                    |                   |          |                   |                        |         |        |            |          |        |

It can be seen from Tables 2 and 3 that the toners in Examples 1 to 20, which were produced through retaining a temperature (°C.) of a dispersion containing a particle of a crystalline polyester resin as a binder resin at Rc-25° C. or higher and Rc-5° C. or lower for 30 minutes or longer in a state where a pH of the dispersion is maintained at 5.5 or higher and 9.0 or lower, each had sufficient low-temperature fixability and suppressed density unevenness of images.

The reason for enhanced low-temperature fixability and suppressed density unevenness of images is not clear. Here, a dispersion containing a toner base particle produced by an emulsion aggregation method in the presence of a metal ion was heat-treated in a specific temperature region while the pH of the dispersion was controlled within a specific range. Because of this, it is considered that an amount of ionic crosslinking which aggregates binder resin fine particles or coloring agent fine particles is controlled within a proper range, and consequently excessive increase in a domain diameter of a crystalline resin and/or bleeding out of the crystalline resin onto a toner surface was prevented.

From the comparison between Examples 1 to 3, and Examples 4 and 5, it is found that low-temperature fixability and suppression of density unevenness of images are more favorably achieved when the temperature of the dispersion during the heat treatment is Rc-25° C. or higher and Rc-10° C. or lower. Moreover, from the comparison between Examples 6 and 7, it is found that low-temperature fixability is further enhanced and density unevenness of images is further lowered when the cooling rate of the dispersion at Rc is 2° C./min or higher. Furthermore, from the comparison between Example 7 and Examples 9 to 12, it is found that low-temperature fixability and suppression of density unevenness of images are more favorably achieved when the pH of the dispersion during heat treatment is 6 to 8.

In contrast, in Comparative Example 1 in which the pH of the dispersion during the heat treatment was 10, low-temperature fixability was found poor although density unevenness of images was favorably suppressed. This is presumably due to the excessively high pH and the resulting increased amount of ionic crosslinking among the binder resin fine particles. Also, in Comparative Example 2 in which the pH of the dispersion during the heat treatment was 4, low-temperature fixability was found poor although density unevenness of images was favorably suppressed. This is

presumably due to the excessively low pH and the resulting dissociation of acid groups in the binder resin and the lowered amount of ionic crosslinking among the binder resin fine particles.

In Comparative Examples 3 and 4 in which the temperatures of the heat treatment in the second step were outside the range of Rc-25° C. or higher and Rc-5° C. or lower, both low-temperature fixability and suppression of density unevenness of images were found poor. This is presumably due to the heat treatment temperatures outside the specific temperature range, and the resulting increased domain diameter of a crystalline resin and bleeding out of the crystalline resin into the vicinity of a toner surface.

In Comparative Example 5 in which heat treatment was not conducted, both low-temperature fixability and suppression of density unevenness of images were poor. Similarly, in Comparative Example 6, image density was uneven. This is presumably because a toner base particle was produced by a suspension polymerization method, not an emulsion aggregation method, and consequently a presence state of a crystalline resin in a toner during the heat treatment could not be controlled.

#### INDUSTRIAL APPLICABILITY

The present invention can provide a toner having excellent low-temperature fixability and low density unevenness of images to be obtained even when a crystalline resin is contained. In addition, the present invention is expected to achieve wider application of a toner as well as further higher performance, higher speed, and energy saving in electro-photographic image forming technology, and the image forming technology will further prevail.

What is claimed is:

1. A process for producing a toner comprising:  
a first step of heating an aqueous dispersion of fine particles of a binder resin, the binder resin comprising an amorphous resin and a crystalline resin, to a temperature higher than or equal to a melting point of the crystalline resin in the presence of a metal ion, whereby the fine particles of the binder resin are aggregated and fused to form a dispersion of toner base particles; and a second step of maintaining the dispersion of the toner base particles at a temperature T (°C.) for 30 minutes

or longer where the dispersion is maintained at a pH of 5.5 or higher and 9.0 or lower, the temperature T satisfying the following expression,  $Rc-25 \leq T \leq Rc-5$ , wherein the  $Rc$  represents a recrystallization temperature ( $^{\circ}$  C.) of the crystalline resin.

2. The process for producing a toner according to claim 1, wherein the temperature T satisfies the following expression,  $Rc-25 \leq T \leq Rc-10$ .

3. The process for producing a toner according to claim 1, further comprising a step of cooling the dispersion to a temperature lower than  $Rc-25^{\circ}$  C. after the aqueous dispersion is heated to a temperature higher than the  $Rc$  in the first step.

4. The process for producing a toner according to claim 1, further comprising a step of cooling the dispersion to a temperature lower than the  $Rc$  at a temperature-lowering rate of  $1^{\circ}$  C./min or higher after the aqueous dispersion is heated to a temperature higher than the  $Rc$  in the first step.

5. The process for producing a toner according to claim 1, wherein the crystalline resin is a crystalline polyester resin.

6. The process for producing a toner according to claim 1, wherein the binder resin is a hybrid resin having an amorphous resin segment and a crystalline resin segment, the amorphous resin is the amorphous resin segment of the hybrid resin, and the crystalline resin is the crystalline resin segment of the hybrid resin.

7. The process for producing a toner according to claim 1, wherein the metal ion is a divalent metal ion.

8. The process for producing a toner according to claim 1, further comprising a step of cooling the dispersion to a

temperature lower than the  $Rc$  at a temperature-lowering rate of  $2^{\circ}$  C./min or higher after the first step and when the aqueous dispersion is at a temperature of  $Rc$ .

9. The process for producing a toner according to claim 1, further comprising a step of cooling the dispersion to a temperature lower than the  $Rc$  at a temperature-lowering rate of  $5^{\circ}$  C./min or higher after the first step and when the aqueous dispersion is at a temperature of  $Rc$ .

10. The process for producing a toner according to claim 1, wherein the pH of the dispersion in the second step is 6.0 or higher and 8.0 or lower.

11. The process for producing a toner according to claim 1, wherein a content of the crystalline resin is 3 to 30 mass % based on the toner.

12. The process for producing a toner according to claim 1, wherein the crystalline resin has a melting point of 50 to  $90^{\circ}$  C.

13. The process for producing a toner according to claim 1, wherein the crystalline resin has a melting point of 60 to  $80^{\circ}$  C.

14. The process for producing a toner according to claim 1, wherein the toner base particles contain an amorphous polyester resin in an amount of 1 to 50 mass %.

15. The process for producing a toner according to claim 1, wherein the toner base particles have a core-shell structure having a shell layer on a core, and the shell layer contains an amorphous polyester resin modified with a styrene-acrylic resin.

16. The process for producing a toner according to claim 1, wherein a content of the crystalline resin in the binder resin is 5 to 50 mass %.

\* \* \* \* \*